

June 29, 1926.

**1,590,603**

E. TAYLOR

## MANUFACTURE OF CELLULOSE PRODUCTS

Filed June 17, 1924



INVENTOR  
Edwin Taylor  
BY  
ward, Crosby & Smith  
ATTORNEYS

## UNITED STATES PATENT OFFICE.

EDWIN TAYLOR, OF BROOKLYN, NEW YORK, ASSIGNOR TO TAYLOR LABORATORIES, INC., OF NEW YORK, N. Y., A CORPORATION OF NEW YORK.

## MANUFACTURE OF CELLULOSE PRODUCTS.

Application filed June 17, 1924. Serial No. 720,524.

My invention relates to improvements in the manufacture of cellulose products and is more particularly illustrated and described hereinafter in its application to the production of cellulose films and similar articles, the apparatus described having particular reference to films or ribbons made from organic material, such as cellulose dissolved in solvents containing a metal such as cupro-  
10 ammonia solution or zinc chloride and from which solutions the organic material is deposited in a solid state upon an anode and the metallic solution-element deposited on a cathode by means of a suitable electrical current.

In carrying out the invention in one form, I pass a metallic belt through an electrical field in a suitable bath the belt constituting the anode upon which the organic material 20 is deposited while the metallic solvent constituent is deposited upon a suitable cathode or cathodes. By this arrangement a continuous film may be produced and its thickness may be governed according to the thickness or density of the solution. Where the belt serves as the anode, the organic material should remain in contact therewith until the last traces of metal have been removed from it. In the apparatus hereinafter described, 30 a suitable belt, not necessarily of great length and preferably of platinum, or platinum plated is caused to pass continuously through a container filled with say for instance, cellulose dissolved in cupro ammonia. By suitable connections this belt which forms the anode carries an electrical current which passes through it and through the cellulose solution or bath to the suitably located cathodes upon which the metallic constituent 40 is deposited. In a preferred form of apparatus, both belt and cellulose solution are moved through the tank or container in the same direction. The electrical current causes the deposition of cellulose upon the belt in a gradually increasing thickness from the point of its first immersion and the cellulose solution is correspondingly reduced in cellulose content and a proportionate amount of solution metal is deposited on the cathodes from which it must be evident that the thickness and density of the deposited film depends upon several factors each of which may be brought fully and conveniently under control of the operator, i. e., the speed 50 of the belt, the time of contact between the

belt and cellulose solution, rate of flow of cellulose solution relative to speed of belt with a consequent variation in strength of the cellulose solution at any point in the tank, and the amount of current passing 60 during any interval of time, etc. In practice, these factors may be so regulated that as the belt emerges from the tank it is coated with a predetermined thickness of cellulose which may then be stripped from the belt 65 in a condition permitting it to be subjected to further operations, or if desired, before stripping it can be scraped to remove surplus adhering material. It may then be passed through a second electrolytic bath, 70 washed, and passed on for further treatment. The cellulose solution reduced in strength by the amount of cellulose deposited from it on the belt, may also be removed, its cellulose content increased such 75 as by methods herein later described, and the concentrated solution returned to the tank. The cathodes may be removed from time to time and the metal which is deposited thereon may be used for the preparation of new cellulose solution. This method 80 it will be observed permits of perfect control of the film thickness and manipulation. It materially reduces the length and cost of the belt (important in some cases where 85 platinum is used) and its subsequent upkeep. The arrangement of the apparatus hereinafter described allows for coating the belt on both sides where this is desired, thereby doubling the output per square foot 90 of one side of belt surface, or where a wheel is employed for casting or flowing the material as in other well known processes. Numerous other advantages will be apparent 95 hereinafter.

In the accompanying drawing forming a part of this specification I have illustrated in vertical section one form of apparatus suitable for carrying out the invention. Referring to the drawing, 1 indicates a closed tank provided with a supply pipe 2 and an outlet 3 provided with a suitable control valve 4. The pipe 3 enters the side of the tank 5 which may be provided with a series of partitions, or walls 6, dividing the tank into several divisions 7, 8, 9 and 10, as shown, so that liquid flowing from the pipe 3 must pass successively through these chambers and finally out of the upper part of the division or compartment 7 of the chamber 110

by way of the overflow pipe 11 which may be provided with a suitable valve such as 12. This overflow enters another tank 13 provided with a draw-off cock 14 and a vent pipe 15 as shown.

An endless belt or carrier 16 which may be made of a suitable copper alloy heavily platinum-plated or preferably of pure platinum, is suitably driven upon the overhead 10 rollers 17, enters the tank 5 passing through the centres of the compartments 7 to 10 inclusive, as shown, being guided and positioned by the rollers 18 in said tank 5 and the small rollers 19. The upper peripheries 15 of the rollers 18 practically contact with the lower extremities of the partitions 6 but a suitable space is left between the lower sides or peripheries of the rollers and the bottom of the tank 5 as shown, so that the liquid 20 may pass freely from one compartment to another from below the lower rollers 18 and over the tops of the upper rollers 19. 20 indicates adjustable soft-edged scrapers adjacent both sides of the belt as it emerges 25 from the tank 5 and serves to remove any adhering material from the films of cellulose deposited upon the belt.

21 indicates a suitable bus-bar or electrical rail connected by the wire 22 to the negative source of electricity 23, and from this bus-bar are suspended a series of copper or other metallic plates 24 so that at least two of them are in each of the compartments 7 to 10 inclusive parallel to and equally distant from the belt 16 and extending downwardly in the tank 10 practically as far as the belt 16. The trolley or rolling contact 25 is connected by a wire 25' to the positive terminal 27 of the same electrical source. 40 Any suitable motive power may be applied to the drive pulley 17 and a pair of brushes, scrapers or other suitable apparatus may be employed as indicated at 26 for cleaning the belt after the film has been stripped therefrom.

In operation, the tank 5 is filled with any desired cellulose solution, such as cupro-ammonia, nickel-ammonia, zinc chloride, etc. Having filled the tank 5 to the level of the 50 outlet pipe 11, the tank 1 is now filled with the same kind of solution, the control valve 4 is opened and a flow of liquid is established through the tank 5, outlet pipe 11, and into the dilute solution tank 13. The belt 55 16 is now started in the direction indicated by the arrow and preferably in a direction parallel with the flow of the cellulose solution and the electric current is turned on. Cellulose will immediately begin to deposit on each side of the belt, becoming thicker and thicker as the belt progresses through the tank 5, the cellulose solution becoming weaker in like proportion, from the point of immersion of the belt in the first compartment to the point of its leaving in the last

compartment. It will be apparent that any variation in the amount of current passed, the speed of the belt through the solution, or the speed of the solution through the tank, will have a corresponding effect on the thickness or quality of the cellulose deposited on the belt and that these factors may be kept under the control of the operator by any well known means. It may be preferable to run the belt rather slowly and to run the solution slightly slower than the belt in order to remove the largest practical amount of cellulose from it before permitting it to flow to the dilute solution in the tank 13. It is unnecessary however to remove all of the cellulose from the solution and it is preferable to keep the solution at a more or less uniform condition and to regenerate or replenish it either by constant inflow of new solution and outflow of partly exhausted solution or by gradual periodic replenishment as may be found preferable according to the particular uses and type of apparatus employed.

After the belt 16 has received the desired thickness of cellulose on both faces, and after the soft-edged scrapers 20 have removed the surplus adhering material from the film thus formed, and have removed or wiped off adhering solution, all of which returns to the tank 5, the belt now passes between the hard-edged scrapers or strippers 28 which separate the film 29-30 from the belt 16, the film 29 passing over the roller 31, directly, and the film 30 passing over the rollers 32-33 which take it out of the path of the returning belt 16 as shown, both films entering the next tank 34 at 35 as shown. This tank 34 is fitted with a suitable outlet valve 36 and a series of guide rollers 37-38. The films 35 pass under and over these rollers traversing the liquid in the tank 34 vertically several times, a slight tension being placed upon the films by means of a driven roller 38' placed in the outer wall 39. 40 indicates a suitable bus-bar connected by the wire 41 to the negative electrical terminal 42, and 43 are the cathodes suspended therefrom. 44 are the anodes suspended from the bus-bar 45 connected by a wire 46 to the positive terminal 47. The tanks 5-34 are covered by a common hood 48 for collecting the vapors which may be drawn off by suction and recovered by way of the outlet 49.

The tank 34 is filled with any solution adapted to remove electrolytically any remaining traces of the metallic solution constituent which may adhere to or be contained in the films or ribbons 29-30. This solution may be a dilute acid such as nitric or sulphuric acid or it may be a normally metallic acid. For some purposes, such as film making, it is preferable to employ a solution of ammonium nitrate as the ultimate product of this salt under electrolysis is

ammonia which by this process is drawn off through the vent pipe 49 and recovered with the ammonia released from the tank 5 when cupro or nickel ammonia solutions of cellulose are employed. The arrangement of anodes and cathodes is such that current passing from one to the other must pass not only through the solution but through the films 28-30 also.

10 The electrolyte in the tank 34 being substantially free of the dissolved organic material or its solution, the film will be greatly purified therein. During treatment and passage through the tank 34 the last trace of 15 metal is removed from the film which now passes over the roll 38' to a wash tank 50. This wash tank is provided with an outlet 51 and valve 52 therefor and with an inlet pipe 53 and valve 54 therefor by means of 20 which a constant flow of liquid is maintained through the tank thereby removing all traces of ammonia or other gases and foreign matter. From the tank 50, the films which pass over the rollers 55 may now be 25 wound upon the reels 56-57 under slight tension, which reels may be removed from time to time as completed. The film thus made is pure cellulose, quite tough and elastic and of a white translucent appearance 30 owing to its content of water. It is however in a suitable condition for further desired operations.

The dilute cellulose solution flowing into the tank 13 is drawn off from time to time, 35 regenerated and returned to the tank 1 for passage through the tank 5. In the case of a cupro ammonia solution, for instance, the liquid in the tank 13 contains cellulose, copper, ammonia and an undue amount of water. This solution may be first cooled, then saturated with ammonia gas after which hydrated cupric-oxide may be added to saturation and finally any desired grade of cellulose also to saturation. The solution may 40 then be filtered, and if desired returned to tank 1, the ammonia and copper used having been obtained largely by recovery from the previous electrolytic action in tanks 5 and 34.

45 The cellulose films upon the reels 56-57 may now be passed over a series of hot rolls if desired and dried. Film thus made can be produced with glass-like transparency and of high tensile strength. It can be adapted to a variety of purposes. It may be cut or 50 otherwise formed in grains nitrated with a mixture of nitric and sulphuric acids, washed, stabilized and dried and an excellent smokeless powder produced without the use of a volatile solvent. By treatment while 55 still slightly moist with a hot solution of nitric acid of about 80% concentration, a material is obtained rather low in nitrogen content but still decidedly soluble in volatile solvents and of value as a waterproof coating for varnish and the like.

For the production of photographic films, a preferred method of treatment is to protect one side of the film by means of a coating of paraffine or by close contact with a revolving drum, and while thus protected 60 to pass the film slowly and continuously through any desired nitrating bath of nitric and sulphuric acid. By this means the surface exposed to the acid is nitrated to any desired depth, the depth of nitrating being 65 controlled by the speed of the film or by the degree of concentration of the acid mixture. The film is now passed through a water bath, the protective coating stripped or otherwise removed (when used) and the film is passed 70 through an electric field between electrodes immersed in a dilute alkaline solution by which means the last traces of acid are readily removed or decomposed. The film is again washed in hot running water and may 75 be dried on hot rolls. It is now passed through a volatile solvent such as acetone or amyl acetate, the non-nitrated side being protected by a drum and the nitrated side gelatinated to the full depth of nitration. The 80 film is now drawn through a drying chamber and the volatile solvent removed. At this stage the product consists of a tough cellulose-like, waterproof backing gradually 85 merging into a non-nitrated water-absorbing facing. The facing is now impregnated with any desired light-sensitive salts, passed 90 through boiling water to improve the sensitivity if desired and finally dried. All 95 of the above operations are continuous, and where space is available the reels 56-57 may be dispensed with and the above operations carried on immediately after the film leaves the roller 55.

In case it is desired to produce an elastic or flexible condition such as may be required for artificial leather, the film after leaving the roll 55 on the wash tank 50 may be led through a solution of glycerine and water, say about thirty per cent (30%) glycerine 100 for about a half hour preferably maintained at a temperature of say about 220° Fahrenheit. This forms a glycerine of cellulose which leaves the film non-hygroscopic under 105 atmospheric conditions.

While the improvements are especially applicable to the treatment of cellulosic materials, they may be usefully applied to other organic materials, such for example as silk which may be dissolved in a nickel ammonia 110 solution to form the electrolyte.

While I have described my improvements in great detail and with respect to preferred embodiments thereof, I do not desire to be limited to such details or embodiments, since many changes and modifications may be made and the invention embodied in widely different forms without departing from the spirit and scope thereof in its broader aspects; hence I desire to cover all modifica- 115

tions and forms coming within the language or scope of any one or more of the appended claims.

What I claim as new and desire to secure 5 by Letters Patent, is:—

1. The method which consists in passing an electrode carrier through an electrolytic cell and causing a solution of organic material to travel through the cell in the same 10 general direction as the carrier but independently thereof, whereby organic material is electrolytically deposited on the carrier from the solution as the two pass through the cell.
15. 2. The method which consists in passing an anode gradually through an electrolytic cell and causing a solution of cellulose to travel through the cell in the same general direction as the anode but independently thereof, whereby cellulose is deposited electrolytically on the anode as the two pass through the cell.
20. 3. The method which consists in passing an electrode through a tank having therein an electrolytic bath containing organic matter in solution while causing the bath to be replenished with organic material.
25. 4. The method which consists in gradually passing an electrode through a tank having therein an electrolytic bath containing cellulose in solution, depositing cellulose on the electrode, while replenishing the bath with fresh cellulosic material.
30. 5. The method which consists in passing a metallic anode carrier through a tank containing an electrolytic bath solution of cellulose whereby cellulose is electrolytically deposited on the carrier, while withdrawing expended electrolyte from one part of the bath and introducing fresh cellulose electrolyte to the bath independently of the carrier.
35. 6. In an apparatus of the class described, an electrolytic cell, a movable electrode traveling through the cell, means for introducing electrolyte at one part of the cell and means for withdrawing expended electrolyte at another part of the cell.
40. 7. In an apparatus of the class described, an electrolytic cell, a movable anode carrier traveling through the cell, means for introducing electrolyte to the part of the cell where the carrier enters the cell, and means for withdrawing expended electrolyte from the part of the cell where the carrier leaves the cell.
45. 8. In an apparatus of the class described, an electrolytic cell, a movable electrode traveling through the cell, means for introducing electrolyte at one part of the cell and means for withdrawing expended electrolyte at another part of the cell and a cathode on both sides of the movable electrode in the cell.
50. 9. In an apparatus of the class described,

an electrolytic cell, a movable anode carrier traveling through the cell, means for introducing electrolyte to the part of the cell where the carrier enters the cell and independently of the carrier, and means for withdrawing expended electrolyte from the part of the cell where the carrier leaves the cell, said carrier being in the form of a metallic belt, and cathodes on both sides of said belt in the cell.

10. In an apparatus of the class described as electrolytic cell, a movable carrier traveling through the cell on which material is electrodeposited in the cell, means for introducing electrolyte at one part of the cell 80 independently of the carrier, and means for withdrawing expended electrolyte at another part of the cell independently of the carrier.

11. The method which consists in passing 85 an electrode carrier through an electrolytic cell containing a solution of organic material whereby organic material is deposited electrolytically on the carrier, and then electrolyzing the organic material in an electrolyte substantially free from said organic material dissolved therein.

12. The method which consists in passing 90 an electrode through an electrolytic bath containing organic matter in solution, whereby organic material is deposited electrolytically on the carrier while causing the cell to be replenished with the organic material, and then electrolyzing the organic material in an electrolyte substantially free from 100 said organic material dissolved therein.

13. The method which consists in passing a carrier continuously through a tank containing an electrolyte with organic material therein, and depositing organic material 105 electrolytically from the solution onto the carrier as it passes through the tank.

14. The method which consists in passing 110 an anode carrier through an electrolytic cell containing a cellulose solution whereby cellulose is deposited electrolytically on the carrier as it passes through the cell, and then treating the cellulose electrolytically in an electrolyte substantially free from dissolved cellulose.

15. The method which consists in passing 115 an anode carrier through an electrolytic cell containing a cellulose solution whereby cellulose is deposited electrolytically on the carrier as it passes through the cell, and then stripping the cellulose from the carrier and passing it between electrodes in an electrolytic cell, the electrolyte in which is substantially free from dissolved cellulose.

16. In an apparatus of the class described, 120 an electrolytic cell, a movable anode carrier traveling through the cell, means for introducing electrolyte to the part of the cell where the carrier enters the cell and independently of the carrier, and means for 125

130

5 withdrawing expended electrolyte from the part of the cell where the carrier leaves the cell, means for stripping off the material deposited on the carrier, a second electrolytic cell and means for conveying said material between the electrodes of said second cell.

17. In an apparatus of the class described, an electrolytic cell, a movable electrode carrier traveling through the electrolyte in the cell, means for stripping off the material deposited on the carrier, a second electrolytic cell and means for conveying said material between the electrodes of said second cell.

18. The method which consists in passing an anode carrier through an electrolytic cell containing a solution of cellulosic material with a metal compound solvent, whereby cellulose is deposited on the anode carrier and the metal is deposited on the cathode of the cell, while the weakened solu-

tion is gradually withdrawn from one part of the cell and fresh solution is introduced into the cell independently of the carrier. 25

19. The method of treating cellulosic material which consists in providing an electrolytic cell with the cellulosic material in solution in the electrolyte therein and subjecting the solution to electrolysis in the 30 cell and adding fresh solution of the cellulosic material while the electrolysis is proceeding.

20. The method which consists in providing an electrolytic cell with cellulosic material in solution in the electrolyte therein, which material is deposited electrolytically on one of the electrodes of the cell, and adding fresh cellulosic material to be electrolyzed, to the electrolyte in the cell while 40 electrolysis is proceeding.

In testimony whereof I have signed my name to this specification.

EDWIN TAYLOR.